

## UNITED STATES PATENT OFFICE

1,972,247

## CONCENTRATION OF OXIDIZED MINERALS

Ralph E. Sayre, Middlesex County, N. J., assignor to American Smelting & Refining Company, a corporation of New Jersey

No Drawing. Application June 20, 1931,  
Serial No. 545,838

29 Claims. (Cl. 209—166)

This invention relates to the concentration of ores and has for an object the provision of an improved process for concentrating oxidized ores.

The present invention is based on my discovery that substances belonging to the class of compounds known as dithiocarbamates may be employed effectively in the concentration of oxidized ores by froth flotation. Dithiocarbamates and their salts such, for example, as their alkali metal salts may be employed in carrying out the process of the invention.

Dithiocarbamates for use in carrying out the process of the invention may be prepared in any suitable manner. In general, the most convenient procedure for preparing such compounds consists in adding an alkali metal sulphide to a mixture of carbon bisulphide and an amine. Thus, for example, sodium a-naphthyl-dithiocarbamate may be prepared by adding sodium sulphide to a mixture of a-naphthylamine and carbon bisulphide.

In order to obtain the reaction product in solid form, it is usually desirable to treat the reaction mixture with ether or with some other solvent in which the dithiocarbamate is but slightly soluble. It is not necessary for the purposes of the present invention to isolate the dithiocarbamate from the reaction mixture. Thus, in the practice of the present invention, the dithiocarbamates may be used as crude reaction products without being isolated from the reaction mixture.

The alkali and alkylammonium salts of substituted dithiocarbamic acids are in general readily soluble in water and alcohol. The heavy metal salts (such as lead, zinc, iron, etc. salts) may be obtained as precipitates by treating the dissolved dithiocarbamates (such as the alkali and alkylammonium dithiocarbamates) with a dissolved salt of the heavy metal. Thus, for example, lead phenyl dithiocarbamate is produced by mixing solutions of lead acetate and potassium phenyl dithiocarbamate. In general, the heavy metal dithiocarbamates are only sparingly soluble even in hot water.

The process of the invention is particularly suitable for the concentration of ores containing silicate and carbonate minerals. In general, the amount of reagent required is from about 0.5 to about 2.0 pounds per ton of dry ore. In treating most ores, a frothing agent such, for example, as pine oil is required.

The reagents may be incorporated in the flotation pulp at any suitable stage of the flotation operation, or they may be added prior to the final wet grinding operation. Relatively pure com-

pounds or products of reactions designed to produce such compounds may be added to the pulp directly or in solution in suitable solvents. Thus, for example, water soluble compounds such as sodium a-naphthyl-dithiocarbamate may be employed in the form of concentrated aqueous solutions.

As a general rule, it is advisable to add the reagent in successive portions at intervals of several minutes until the required amount has been added. The use of a filming agent such as sodium sulphide is sometimes desirable, and it is preferably added in successive portions at or immediately preceding the times at which the dithiocarbamate additions are made. In carrying out the process of the invention, neutral and alkaline pulps may be employed. In general, the use of a slime-conditioning agent such as lime or sodium silicate is advantageous. Such agents may be added, conveniently, prior to the final wet grinding of the ore.

The following examples give typical results obtained in the treatment of ores containing copper and lead silicate and carbonate minerals:

## Example I

A 500 gram sample of Mason Valley copper ore containing practically all of its copper in the form of malachite and chrysocolla was ground with water to produce a pulp in which 89.4 percent of the particles were minus 200 mesh. The resulting pulp was subjected to a froth flotation operation for a period of 20 minutes in a Janney laboratory flotation machine.

The quantities of reagents employed and the results obtained were as follows:

| Reagents                                                   | Lbs. per ton of dry ore |                  | 95  |
|------------------------------------------------------------|-------------------------|------------------|-----|
|                                                            | Percent Cu              | Percent recovery |     |
| Sodium a-naphthyl-dithiocarbamate.....                     | 1.6                     |                  |     |
| Sodium silicate.....                                       | 2.0                     |                  |     |
| Sodium sulphide (Na <sub>2</sub> S·9H <sub>2</sub> O)..... | 2.0                     |                  |     |
| Pine oil.....                                              | 0.07                    |                  |     |
| Heads.....                                                 | 3.38                    |                  | 100 |
| Concentrates.....                                          | 15.07                   | 77.8             |     |
| Tailings.....                                              | 0.91                    |                  |     |

## Example II

A 500 gram sample of Copper Basin copper ore containing practically all of its copper in the form of malachite and chrysocolla was ground with water to produce a pulp in which 85.2 per-

cent of the particles were minus 200 mesh. The resulting pulp was subjected to a froth flotation operation for a period of 15 minutes in a Janney laboratory flotation machine.

5 The quantities of reagents employed and the results obtained were as follows:

| Reagents |                                         | Lbs. per ton of dry ore |                  |
|----------|-----------------------------------------|-------------------------|------------------|
| 10       | Sodium a-naphthyl-dithiocarbamate       | 2.0                     |                  |
|          | Sodium silicate                         | 3.0                     |                  |
|          | Sodium sulphide ( $Na_2S \cdot 9H_2O$ ) | 2.0                     |                  |
|          | Pine oil                                | 0.14                    |                  |
| 15       |                                         | Percent Cu              | Percent recovery |
|          | Heads                                   | 2.40                    |                  |
|          | Concentrates                            | 9.12                    | 67.1             |
|          | Tailings                                | 0.95                    |                  |

20

### Example III

A 500 gram sample of Miami copper ore containing practically all of its copper in the form of chrysocolla was ground with water to produce a pulp in which 84.3 percent of the particles were minus 200 mesh. The resulting pulp was subjected to a froth flotation operation for a period of 12 minutes in a Janney laboratory flotation machine.

30 The quantities of reagents employed and the results obtained were as follows:

| Reagents |                                         | Lbs. per ton of dry ore |                  |
|----------|-----------------------------------------|-------------------------|------------------|
| 35       | Sodium a-naphthyl-dithiocarbamate       | 1.0                     |                  |
|          | Sodium silicate                         | 1.0                     |                  |
|          | Sodium sulphide ( $Na_2S \cdot 9H_2O$ ) | 1.0                     |                  |
|          | Pine oil                                | 0.14                    |                  |
| 40       |                                         | Percent Cu              | Percent recovery |
|          | Heads                                   | 1.75                    |                  |
|          | Concentrates                            | 10.81                   | 74.9             |
|          | Tailings                                | 0.50                    |                  |

45

### Example IV

A 500 gram sample of Utah Copper Company copper ore containing practically all of its copper in the form of malachite and azurite was ground with water to produce a pulp in which 75.2 percent of the particles were minus 200 mesh. The resulting pulp was subjected to a froth flotation operation for a period of 15 minutes in a Janney laboratory flotation machine.

55 The quantities of reagents employed and the results obtained were as follows:

| Reagents |                                         | Lbs. per ton of dry ore |                  |
|----------|-----------------------------------------|-------------------------|------------------|
| 60       | Sodium a-naphthyl-dithiocarbamate       | 1.2                     |                  |
|          | Sodium silicate                         | 1.0                     |                  |
|          | Sodium sulphide ( $Na_2S \cdot 9H_2O$ ) | 1.0                     |                  |
|          | Pine oil                                | 0.14                    |                  |
| 65       |                                         | Percent Cu              | Percent recovery |
|          | Heads                                   | 1.81                    |                  |
|          | Concentrates                            | 13.47                   | 77.5             |
|          | Tailings                                | 0.46                    |                  |

70

### Example V

Another 500 gram sample of the Utah Copper Company ore, in a pulp corresponding to that employed in Example IV, was subjected to a similar

flotation operation for a period of 20 minutes in the absence of sodium sulphide and in the presence of lime and an increased amount of sodium a-naphthyl-dithiocarbamate.

80 The quantities of reagents employed and the results obtained were as follows:

| Reagents |                                   | Lbs. per ton of dry ore |      |
|----------|-----------------------------------|-------------------------|------|
|          | Sodium a-naphthyl-dithiocarbamate | 2.0                     |      |
|          | Lime ( $Ca(OH)_2$ )               | 0.3                     |      |
|          | Pine oil                          | 0.14                    |      |
|          | Percent Cu                        | Percent recovery        |      |
|          | Heads                             | 1.81                    |      |
|          | Concentrates                      | 13.47                   | 76.7 |
|          | Tailings                          | 0.47                    |      |

### Example VI

A third 500 gram sample of the Utah Copper Company ore, in a pulp corresponding to that employed in Example IV, was subjected to a similar flotation operation for a period of 20 minutes in the absence of sodium sulphide and in the presence of sodium silicate and an increased amount of sodium a-naphthyl-dithiocarbamate.

100 The quantities of reagents employed and the results obtained were as follows:

| Reagents |                                   | Lbs. per ton of dry ore |      |
|----------|-----------------------------------|-------------------------|------|
|          | Sodium a-naphthyl-dithiocarbamate | 2.0                     |      |
|          | Sodium silicate                   | 1.0                     |      |
|          | Pine oil                          | 0.14                    |      |
|          | Percent Cu                        | Percent recovery        |      |
|          | Heads                             | 1.81                    |      |
|          | Concentrates                      | 13.39                   | 83.8 |
|          | Tailings                          | 0.33                    |      |

### Example VII

A 500 gram sample of Yellow Pine lead ore containing practically all of its lead in the form of cerussite was ground with water to produce a pulp in which 89.2 percent of the particles were minus 200 mesh. The resulting pulp was subjected to a froth flotation operation for a period of 15 minutes in a Janney laboratory flotation machine.

120 The quantities of reagents employed and the results obtained were as follows:

| Reagents |                                         | Lbs. per ton of dry ore |      |
|----------|-----------------------------------------|-------------------------|------|
|          | Sodium a-naphthyl-dithiocarbamate       | 0.6                     |      |
|          | Sodium sulphide ( $Na_2S \cdot 9H_2O$ ) | 6.0                     |      |
|          | Pine oil                                | 0.14                    |      |
|          | Percent Pb                              | Percent recovery        |      |
|          | Heads                                   | 6.67                    |      |
|          | Concentrates                            | 40.20                   | 77.3 |
|          | Tailings                                | 1.51                    |      |

130 In each of the tests reported above, a pulp containing about 20% solids by weight was employed. The slime conditioning agents such as lime and sodium silicate were added to the pulp during the grinding operations. The remaining reagents were added in small amounts at short intervals during the course of the flotation operations.

75

145

150



chrysocolla which comprises subjecting the ore in the form of a pulp to a froth flotation operation in the presence of a slime conditioning agent and an alkali metal dithiocarbamate.

5 26. The process of concentrating oxidized ore containing one or more minerals of the group consisting of malachite, azurite, cerussite and chrysocolla which comprises subjecting the ore in the form of a pulp to a froth flotation operation in the presence of a sulphide filming agent, a slime conditioning agent and an alkali metal dithiocarbamate.

10 27. A process of concentrating oxidized ore containing the mineral malachite, which com-

15

prises subjecting the ore in the form of a pulp to a froth flotation operation in the presence of an alkali metal dithio-carbamate.

28. A process of concentrating oxidized ore containing the mineral cerussite, which comprises subjecting the ore in the form of a pulp to a froth flotation operation in the presence of an alkali metal dithio-carbamate.

80 29. A process of concentrating oxidized ore containing the mineral chrysocolla, which comprises subjecting the ore in the form of a pulp to a froth flotation operation in the presence of an alkali metal dithio-carbamate.

85 RALPH E. SAYRE.

90

20

95

25

100

30

105

35

110

40

115

45

120

50

125

55

130

60

135

65

140

70

145

75

150